

# UNITED STATES PATENT OFFICE.

WILLIAM G. HUGHES, OF PITTSBURGH, PENNSYLVANIA.

## INCANDESCENT BODY FOR ELECTRIC LAMPS.

1,106,384.

Specification of Letters Patent. Patented Aug. 11, 1914.

No Drawing.

Application filed December 16, 1912. Serial No. 737,038.

To all whom it may concern:

Be it known that I, WILLIAM G. HUGHES, a citizen of the United States, and residing at Pittsburgh, in the county of Allegheny and State of Pennsylvania, have invented new and useful Improvements in Incandescent Bodies for Electric Lamps, of which the following is a specification.

The invention has for its object the production of an incandescing filament for incandescent electric lights or lamps which is composed of substantially pure uranium.

Another object of my invention is to provide a filament of a tough fibrous nature which will be less liable to fracture than filaments composed of material which is of a brittle granular nature.

A still further object of my invention is to provide a filament composed of a material which by reason of its peculiar nature will afford increased candle power in the lamp with less consumption of current.

Incandescent filaments in accordance with my invention may be manufactured in accordance with different processes, the preferred one of which will be hereinafter described.

In accordance with the preferred process for obtaining the metallic uranium, I take, in substantially proportions herein given, uranium chlorid 75 grains, metallic sodium (finely divided) 50 grains, and potassium chlorid 150 grains. I place these substances, in layers, in a porcelain or alundum crucible, and cover the crucible contents with potassium. I then place this crucible with its contents in an iron crucible of a size to provide a space between the two crucibles, and I fill this space between the inner and outer crucible with clean broken or granular carbon. I then seal the iron crucible and subject the whole to a high temperature sufficient to produce a white heat. This sets up a thermo-chemical action with the result that the metallic uranium is formed or settles in the bottom of the inner crucible. After obtaining the uranium metal, it is then annealed by any suitable annealing

process, in the absence of air, after which it is drawn into wire by any of the well-known processes by which it is shaped for filament use. As an example of one method of annealing and one of drawing the uranium, the following is given. In annealing, the uranium is brought to a high temperature, say 2000° C., either *in vacuo*, or in an atmosphere of a neutral gas, or in a space from which atmospheric air has been practically exhausted, and is then permitted to cool under the same conditions. When cold, and thus annealed, the uranium which is in pure metallic form, is drawn into a filament by first passing it through grooved rolls to reduce it to wire-like form, is then re-annealed in any preferred manner, as for example, by the procedure above outlined and is then drawn through suitable dies, the final or finishing die being constructed from a diamond or other suitable jewel.

In accordance with my invention, the filament is composed solely of dense coherent metallic uranium having an extremely high fusing point and capable of great incandescent efficiency at a comparatively low watt rate per candle power, and free from perceptible disintegration at such efficiency.

Having fully described my invention, what I claim is:—

1. A filament for incandescent lights composed of drawn uranium in pure metallic state.
2. A filament for incandescent lights composed of annealed and drawn uranium in pure metallic state.
3. A preliminary product to be used in the production of incandescent filaments consisting of uranium chlorid, metallic sodium, and potassium chlorid in substantially the proportions specified.

In testimony whereof I affix my signature in presence of two witnesses.

WILLIAM G. HUGHES.

Witnesses:

IDA L. CHERRELL,  
TONA WAGNER.